

May 5, 1925.

1,536,952

S. M. UDALE ET AL.

METHOD OF PROTECTING THE SURFACES OF METAL MOLDS.

Filed May 6, 1922



*Stanley M. Udale*  
*Samuel H. Meloche*  
INVENTORS.

## UNITED STATES PATENT OFFICE.

STANLEY M. UDALE AND DANIEL H. MELOCHE, OF DETROIT, MICHIGAN, ASSIGNEES TO  
GEORGE M. HOLLEY, OF DETROIT, MICHIGAN.

## METHOD OF PROTECTING THE SURFACES OF METAL MOLDS.

Application filed May 6, 1922. Serial No. 559,076.

To all whom it may concern:

Be it known that we, STANLEY M. UDALE, and DANIEL H. MELOCHE, citizens of the United States, residing at 893 Lothrop 5 Ave., and 8450 Fourteenth St., Detroit, in the county of Wayne and State of Michigan, have invented certain new and useful Improvements in Methods of Protecting the Surfaces of Metal Molds, of which the following is a specification.

This invention relates to improved means for the protection of surfaces of metal molds used in the continuous production of metal castings. This invention consists 15 essentially in the application to a permanent mold of a refractory coating applied by means of a blow torch.

The molds are preferably made of cast iron and the chief object of this invention 20 is to provide means for the protection of the surfaces of such molds when used for the production of grey iron castings.

The actual method practiced by the applicant is shown in the figure, in which a 25 pipe A is connected to a regulable supply of oxygen and acetylene. The pipe A is threaded into the casing B, which is preferably lined with a refractory coating. Air entrances C and D may be provided as 30 required. A depression E is located in the casing B forming a crater. Opposite this crater E is the opening F, through which the refractory powder is fed into the crater E. The casing B and crater E are 35 protected by a refractory lining G. The amount of oxygen and the area of the air openings C and D are regulated so that an intensely hot flame results. H represents a permanent master positive mold 40 which is to be protected by means of a refractory coating.

The flame is directed against the mold H and as the refractory powder is highly heated as it travels toward the mold through the flame it therefore arrives at the mold in a highly heated state and as the mold is also heated by the flame directed upon it, the refractory substance adheres to the mold. The refractory particles, which are 45 very finely divided, are at a white heat when they strike the heated mold, which accounts for the fact that they do adhere firmly enough so as to protect the molds 50

during repeated use. Moreover, the iron is softened slightly by the heat, whereas the 55 hardness of the refractory particles is not appreciably diminished.

In actual use the life of the refractory coating is extended by protecting it with a layer of lamp black applied in a well 60 known manner by means of a smoky flame.

The refractory substances which we have found most satisfactory are stannic oxide and magnesium oxide.

The function of the crater G is to catch 65 particles not carried directly into the flame, heat these particles and by means of the violent eddy in this crater to return these particles to the flame.

What we claim is:

1. The means for protecting the surface 70 of permanent metal molds in which metals are cast, having a casting temperature in excess of 2000° F., which consists in subjecting the surface of the mold to the action 75 of a blow torch, to the flame of which a refractory powder is fed.

2. The method of protecting the metal 80 surface of permanent metal molds to be used in the production of metal castings which consists in coating the surface of 85 metal molds with a refractory non-volatile metallic oxide, the metallic oxide being applied in powdered form within the flame of a blow torch directed against the surface 85 of the permanent iron mold.

3. The method of protecting the metal 90 surface of permanent iron molds which consists in heating the surface of the mold by a blow torch directed against the surface 90 and injecting into said flame a refractory powder.

4. The method of protecting the metal 95 surface of permanent iron molds, which consists in heating the surface of the iron molds by means of the flame of a blow torch directed against the surface of the said molds and injecting into the flame powdered stannic oxide whereby the particles of stannic oxide are carried against the surface 100 of the iron molds which are thereby coated with the stannic oxide.

In testimony whereof we affix our signatures.

STANLEY M. UDALE.  
DANIEL H. MELOCHE.